

# UNITED STATES PATENT OFFICE.

FRANK J. BAUMGARDNER, OF CLEVELAND, OHIO, ASSIGNOR OF ONE-FOURTH TO FRANK L. PHIPPS AND ONE-FOURTH TO CHARLES R. GIBSON, BOTH OF CLEVELAND, OHIO.

## PAPER-STOCK.

1,334,513.

Specification of Letters Patent. Patented Mar. 23, 1920.

No Drawing. Application filed March 3, 1917. Serial No. 152,248. Renewed August 6, 1919. Serial No. 315,787.

*To all whom it may concern:*

Be it known that I, FRANK J. BAUMGARDNER, a citizen of the United States, residing at Cleveland, in the county of Cuyahoga and 5 State of Ohio, have invented certain new and useful Improvements in Paper-Stocks, of which the following is a specification.

My invention relates to improvements in paper-stocks, the primary object being the 10 provision of a generally improved paper-stock whereby a generally improved paper having the particular qualities required to meet the varying demands of actual service may be produced from paper-pulp prepared 15 in any suitable and convenient manner from any of the usual and well known pulp forming materials.

More specifically stated, my invention relates to an improved filler or "engine sizing" 20 adapted to be used in lieu of and as an improved substitute for certain materials or chemicals, such for example, as China clay, alum, sulfate of soda, resin, and the like, now commonly employed for such purposes 25 and which have been found objectionable for reasons hereinafter pointed out.

My improved filler comprises powdered or 30 finely divided oyster shells reduced by grinding or crushing and preferably of a fineness adapted to pass through a screen of from (250) two hundred and fifty to (300) three hundred mesh per square inch according to 35 the particular nature of the prepared pulp and the material from which it is reduced as well as the requirements of the particular 40 paper to be produced. Suitable sizing material in comparatively small proportion may also be incorporated therewith for smoothing the printing surface where such 45 is required in the paper to be produced, and my improved filler is preferably thoroughly incorporated with the prepared pulp in substantially the proportions of (1) one part of such filler to five (5) parts of pulp, and 50 such proportions being best obtained by weighing the pulp and filler material so that for example (5) five pounds of the former will be present to (1) one pound of the latter, such proportions, however, being varied somewhat in accordance with the nature of 55 the pulp and the character of the paper to be produced.

In carrying out my invention, the improved filler is preferably introduced as a

step in the process of preparing the paper-stock for use in the paper making machine, and is preferably introduced into the pulp as it comes from the reducing or beating engine and while such pulp is in the mixing or washing engine so that such pulp will 55 become thoroughly impregnated with such powdered oyster shells (and surface sizing where such is used) in about the proportions stated, and preparatory to introduction 60 into the machine.

I have discovered that such powdered shells when introduced and combined as stated furnish what is supplied by the above mentioned commonly employed eliminated 65 chemicals and that the same eliminates the undesirable properties and objections thereto as found by actual experience and well known to those skilled in this particular art.

For example,—China clay fills the pores 70 of the paper and renders it brittle and more liable to break or tear. Alum is used as a precipitating agent and as this filler is itself a precipitant this ingredient may be readily dispensed with. Sulfate of soda is unnecessary as its qualities are made up in the 75 improved filler and, furthermore, owing to the calcium silicates contained in this filler a strong binding agent or medium is provided thereby making the resultant paper 80 stronger and more flexible, holding its consistency at all times and rendering the same 85 absolutely free from acids.

Furthermore, the chlorid of lime used as a 90 bleaching agent in the preparation of the pulp afterward gives off from the paper produced a noxious odor which latter is largely eliminated by the improved filler and owing to the particular character and properties of the same in many cases the use 95 of chlorid of lime or other bleaching agent may be largely reduced and in some cases entirely dispensed with.

Practical experiments and tests have 100 shown that the paper resulting from the use of my improved paper filler is stronger in proportion to weight, has a better surface with improved ink-taking qualities, and is less affected by moisture.

By the use in the paper pulp of my improved filler as a strengthening and binding 105 agent, the liability of the paper to break between the cylinders on the Webb presses is reduced to a minimum. The paper being

more thoroughly impregnated with the filler is less porous and consequently gathers less moisture.

Furthermore, many of the materials now used in the manufacture of paper have a marked abrasive action on the wire screens of paper-making machines whereas by the use of this improved filler, such abrasive action is entirely eliminated.

- 10 Furthermore, on high grade coated paper a trouble often encountered is a loosening of the coating of baryta and which does not result from paper produced through the use of my improved paper-stock.
- 15 Having thus described my improved paper-stock, without having attempted to set forth all the forms in which it may be made, or all the modes or applications of its use, what I claim and desire to secure by Letters

20 Patent, is,—

1. An engine sizing for paper-pulp, comprising finely divided oyster shells.

2. A paper made from paper pulp and finely divided oyster shells.

3. A filler for paper-stock, comprising 25 finely divided oyster shells and a sizing material.

4. A composition for paper-stock, comprising paper-pulp and powdered oyster shells.

5. A composition for paper-stock, comprising paper-pulp and finely reduced oyster shells combined in substantially the proportions stated.

6. A composition for paper-stock, comprising paper-pulp and powdered oyster shells in about the proportions of five (5) parts of the former to one (1) of the latter.

In testimony whereof I have affixed my signature in the presence of two witnesses. 40

FRANK J. BAUMGARDNER.

Witnesses:

F. L. PHIPPS,  
CHAS. R. GIBSON.